

## UNITED STATES PATENT OFFICE

2,417,833

## LUBRICANT

Bert H. Lincoln and Joseph M. Hersh, Ponca City,  
Oklahoma, assignors to Continental Oil Company,  
Ponca City, Oklahoma, a corporation of Delaware

No Drawing. Application April 22, 1944,  
Serial No. 532,346

9 Claims. (Cl. 252—33.6)

1

Our invention relates broadly to lubricants and more particularly to the use of the higher aliphatic diacids having terminal carboxyl groups as a base material for introducing into the lubricant chemical elements or groups which have a beneficial effect thereon.

Most lubricating oils are deficient in one or more respects. They may have a low resistance to oxidation, corrosion, foaming or sludge formation or low detergency, oiliness or extreme pressure characteristics. It has become the general practice to add to the oil small amounts of an agent or agents capable of correcting or at least minimizing the deficiency. The additives are chemical compounds but it is usually one element or radical in the compound which produces the desired result. These elements, radicals and compounds, are well recognized in the art and have been generally classified according to the result they produce in the lubricant.

For example, low resistance of a lubricant to corrosion, oxidation and sludge formation is corrected by the use of sulfur, phosphorous and nitrogen compounds. Sulfurized sperm oil, sulfurized wax olefins, organic thiophosphates and thiocarbonates, and aromatic or amino-aromatic phosphates are typical examples. As little as 0.001 per cent of these compounds is usually sufficient.

Foaming of lubricants can be corrected by the addition of .0001 per cent or less of certain active organic silicon compounds such as aliphatic silicone oils, silicone resins or aryl alkyl silicane derivatives.

Improvement in detergency is effected by the addition to the oil of compounds capable of dispersing, peptizing, or suspending sludge-forming materials therein. Metal salts of petroleum sulfonic acids, metal salts of alkyl substituted phenols and thiophenols, metal salts of phosphoric or thiophosphoric acid, metal salts of organo substituted fatty acid esters and tin, zinc, barium, calcium, aluminum, sodium, potassium and lithium salts and soaps of various organic acids and hydroxy compounds are classes of compounds commonly used as detergents. Typical specific examples of these classes are calcium sulfonate, calcium phenyl stearate, zinc thiophosphate esters and calcium dichlorostearate. From 0.1 per cent to 10 per cent of the detergent additive is generally required depending upon the activity of the specific additive employed.

Oiliness and extreme pressure characteristics of lubricants are improved by the addition of chlorinated or sulfurized fatty acid esters or chlorinated wax, in concentrations ranging from 0.01 per cent to 1.0 per cent. Methyl dichloro-

2

stearate, sulfurized sperm oil, trilauryl phosphate and oleic acid are specific examples.

An important object of our invention is to provide an additive that will materially increase the beneficial effect of these compounds on the lubricant.

Another object of our invention is to provide an additive that combines one or more functional groups of the above compounds in a single molecule.

Other objects and advantages of our invention will be apparent during the course of the following description.

We have discovered that the efficiency of these compounds or radicals can be increased to an unexpected degree by introducing them as substituents of an aliphatic diacid of from 6 to 12 carbon atoms having terminal carboxyl groups. Although any of the acids included in this group may be used, we prefer azelaic acid,



The diacids can be prepared commercially by a controlled oxidation of the corresponding unsaturated fatty acid with ozone, peroxides, permanganates or nitric acid. For example, azelaic may be prepared by the controlled oxidation of oleic acid with ozone.

The outstanding superiority of the substituted diacid may be attributed to the fact that it is a dipolar molecule. The terminal carboxyl groups are apparently balanced and spaced by the intermediate aliphatic chain and their presence at each end of the chain permits the molecule to be oriented in relation to a lubricated surface. This theory accounts for the fact that the same results are not observed if the active radicals are substituted on an acid having but one carboxyl group or on a diacid having proximal or non-terminal carboxyl groups. The molecular structure of the latter acids does not permit orientation of both polar carboxyl groups with respect to a planar surface without molecular strain.

We have found that certain compounds are adsorbed or absorbed on the surface of metals in the form of a plurality of layers. This "built up" or "compound" film is very tenacious and has the property of very markedly reducing the coefficient of friction. The compounds most readily adsorbed by metals are ones consisting of polar molecules, that is, molecules of unsymmetrical electrical character which contain an atom or group of atoms exhibiting a secondary or residual valence. These polar compounds tend to produce regimentation of the molecules of hydrocarbon oil when added thereto. If a metal is immersed in a strongly polar compound, a regi-

imentation or cybotaxis of the molecules will take place in the adsorbed film, the molecules being oriented with respect to the surface of the metal by which they are adsorbed.

We have found that oil soluble polar molecules having more than one polar group show exceptionally good or poor adsorption properties depending upon the nature and position of the polar groups. It is in this connection that the azelaic acid derivatives are particularly effective, since polarity developed in azelaic esters or salts due to the halogen substitution on the alpha carbon (the carbon atom adjacent the carboxyl group) is enhanced by the concomitant polar group substituted on the sixth carbon atom in the molecule, which spacing is ideally suited for synergistic action in accord with the concept of carbon-carbon valence angles and the known ease of formation of six carbon ring systems.

Conversely, dicarboxylic acids having non-terminal carboxyl groups have an opposite effect due to the steric hindrance of its asymmetric molecule just as diacids of less than six carbon atoms have noncomplimentary polar groups due to the strain inherent in forming an adsorbed ring of less than four carbon atoms.

While the above theory offers a logical explanation for the superiority of the substituted compound embodying the invention, it is to be understood that we are not bound by it. Our claims are based upon the superior results observed and not upon any theory to support it.

Another important characteristic of the acid molecule is its ability to form a stable compound with a number of different functional radicals substituted thereon. These radicals can be substituted on both the terminal carboxyl groups and the connecting aliphatic chain. The molecule is thus able to bring all of the substituted radicals into intimate association with the lubricant and the lubricated surface. This is important since a radical which has a beneficial effect upon one characteristic of the lubricant may impair some other desirable characteristic. The adverse effect can be obviated by substituting another element or group on the acid molecule that will enhance the impaired characteristic. In a sense the two radicals complement each other. It is further interesting to note that the complementary radicals are more effective when introduced into the lubricant as part of the same diacid molecule than when introduced as separate compounds according to conventional practice. Under different circumstances it is, of course, necessary to substitute various radicals or combinations of radicals on the diacid molecule.

The amount of the substituted diacid that must be mixed with a lubricant to obtain maximum correction of its deficiencies will depend upon the particular characteristics that are deficient and upon the particular radical or combination of radicals with which the acid is substituted. We have found that amounts in the order of from 0.0001% to 10% are usually sufficient. In every instance amounts less or more than the optimum amount can be used with less satisfactory results. If the additives are used in relatively high concentrations of from 0.1% to 10%, compounds should be selected that are readily miscible with the lubricant. If lower concentrations of from 0.0001% to 0.1% are used, less soluble compounds may be used since high oil solubility is not such a critical factor.

We have found that the following classes of substituted diacids have high utility.

*1. Mono- or diacid salts*



In the above formula "M" is a salt forming element such as the metals calcium, barium, strontium, tin, zinc, chromium, cobalt, aluminum, sodium, potassium, lithium, magnesium, bismuth, copper, nickel, manganese, cadmium or silver, or a salt forming group such as ammonium or an amine; and "R" and "R<sub>n</sub>" are organic radicals, there being one or more such R groups as shown by the subscript numerals. As shown, one or both of the terminal carboxyl groups may be neutralized by a salt forming element or radical.

When a monovalent element or radical is used in the above formula, compounds of the following type are obtained.

- 25 1. Lithium alpha-dichlor-methyl azelate.
- 25 2. Sodium 8-chloro-8-ethylxanthyl ethyl azelate.
- 30 3. Ammonium phenyl chloro-azeloyl thiocarbonate.
- 30 4. Diethyl-ammonium azeloyl diphenyl silicol.
- 30 5. Sodium anilino-8-chloro-8-diethyl thiophosphate-azelate.
- 35 6. Diphenyl-ammonium 8,8-dicresyl ethyl azelate.
- 35 7. Lithium anhydro-diazeloyl anilide.

When a polyvalent element or radical is used any of the following types of compounds may be obtained depending upon the particular element or radical selected and conditions under which the substitution takes place.

40 A. Intramolecular diacid salts of the type shown under (1) below if "M" is a bivalent element or radical, or of the type shown under (2) below if "M" has a valence greater than two.



60 In the second formula shown above (OOCR) is an aliphatic acid group; (O—R') is an aromatic acid group; (OX) is an inorganic acid group; (R) is an aliphatic group; (R') is an aromatic group; and "n" is an integer equal to the "M" valence minus two. The following compounds are typical of those included in the Formula IA (1) and IA (2) above:

- 65 1. Alpha-dichlorostearyl-aluminum azelate.
- 65 2. Cresyl-thallium 8-dibutyl phosphato-azelate.
- 70 3. Di-p.-chlorophenoxy-tin azelate.
- 70 4. P.-ethyl phosphitophenyl-aluminum 8-diethylxanthyl azelate.
- 75 5. Diethyl-tin azelate.
- 75 6. Phenyl-thallium azelate.

7. Alpha-naphthyl-chromium 8 - dichloro-azelate.

B. Intermolecular mixed salts of the type shown in the following formula:



where M and M' are the same or different metals having valences of two or more and R and R<sub>2</sub> are organic radicals, there being one or more such R groups as shown by the subscript numbers. The groups linked through "n" to the diacid molecule may be aliphatic or aromatic organic acid radicals, inorganic acid radicals or alkyl or aryl hydrocarbon radicals.

Typical examples of compounds included by 20

Formula IB are:

1. Alpha-chlorostearyl-bismuth 8 - di - butylxanthyl ethyl azelate.

2. Triphenyl-tin ethyl 8-dichloro-azelate.

3. Calcium di (8,8'-dichloro-ethylxanthyl) p-25 chloro-anilino-azelate.

4. Dibutyl - phosphato - zinc alpha naphthyl-azelate.

5. Zinc di- (8,8' dibutyl thiophosphato) thiophenyl azelate.

### II. Mono- or diacid esters



where R and R' are organic radicals such as the 40 simple or substituted mono, di, or poly-hydroxy alkyl, cyclo-alkyl or aryl-alkyl radicals, simple or substituted mono or poly-cyclic aryl or alkyl-aryl derivatives or simple or substituted heterocyclic derivatives.

Typical examples of compounds included in the Formula II above are:

1. Lauryl dichlorostearyl azelate.

2. Sodium dichloro-ricinoleyl azelate.

3. Calcium di (dibenzyl) azelate.

4. Zinc di - (8,8' - diphenyl) p.-chlorophenyl 50 azelate.

5. Cyclohexyl 8-chloro-8-ethylxanthyl ethyl azelate.

6. Alpha - naphthyl 8-di-p-chlorophenyl ethyl 55 azelate.

7. Dithiofurfuryl 8 - dithiobutyl thiophenyl azelate.

8. 3,5 - diamylphenyl 8 - diethylthiophosphato-60 sodium azelate.

### III. Mono- or diamide of imide derivatives

This class of compounds is divided roughly into two groups as shown in Formulas A and B below.

A.



of the class of compounds defined by Formula A:

1. Sodium alpha-dithiophenyl azeloyl diphenyl amide.

2. Alpha-dichloro methyl azeloyl phenyl hydrazide.

3. Calcium di- (alpha-diphenyl) tributyl-siliconamido azelate.

4. Lauryl alpha-di-p.-hydroxyphenyl azeloyl-phenyl azide.

5. Stearyl calcium alpha-di-(dibutyl phosphate) tricyclohexyl-silicon azeloyl amide.

B.



In the above formula the amide or imide nitrogen may be unsubstituted or have substituents such as:

a. Organic substituents R or R',

b. Hydrazo radical —NHR,

c. Hydrazine radical —NH<sub>2</sub>,

d. Nitrile —CN.

The following compound is a typical example of the class of compounds defined by Formula B.

1. Alpha-diethylxanthyl azeloyl - imido-silicon triphenyl.

### IV. Derivatives of azelaic anhydride



OM, OR, NH<sub>2</sub>, ONH<sub>2</sub>

As shown by the above formula the mono, di or polymolecular acid anhydrides or their derivatives may be formed:

A. The anhydride may be decarboxylated on heating to produce a cyclic ketone, azelaone, as shown in the following formula:



This cyclic compound may further be reduced to the cyclic alcohol to form alcoholates, ethers or esters.

B. The anhydride may react with organo-silicates, organo-carbonates or thiocarbonates producing an azelaic ester silicate or carbonate as shown in the following formula:



C. The anhydride may react with alcohols,

phenols or thiophenols to produce the organic esters. Typical examples of such esters are:

1. Calcium di-(alpha-chloro, alpha-thiophenyl) azelaic anhydride.
2. Zinc di-(alpha-dicresyl) cyclooctyl thio-phosphate.
3. Calcium di-(alpha diethylxanthyl) cyclo-octyl stearate.
4. Methyl dichloro-azeloyl tributyl silicane.
5. Lauryl di-ethylxanthyl ethylxanthyl azelate.
6. Lithium alpha-dithiophenyl thiocresyl azelate.

#### V. Derivatives of dithiolic acid



A. Azeloyl dithiolic acid forms metal salts, esters or anhydrides in the same manner as the oxy-acid.

B. The disulfide or the original acid or its derivatives may be further sulfurized with either elemental sulfur or a sulfur compound to form poly-thio acids and their derivatives as shown by the following formula:



Typical examples of poly-thio acid derivatives are:

1. Lithium alpha-diphenyl p.-chlorophenyl dithio-azelate.
2. Alpha di-ethylxanthyl azeloyl disulfide.
3. Dithiophenyl 2, 8-dichloro 2,8-dithiobutyl azelate.
4. Methyl dichlorostearyl alpha dichloro-di-thio-azelate.

#### VI. Derivatives of alpha halogen azelates



In the above formula the (\*) represents active atom positions for halogenation; X represents any halogen. Mono or dihalide substitutions can be produced on either or both of the active carbons.

a. The halogen atoms may be replaced by alkyl or aryl groups by use of the Friedel-Crafts' reaction with aluminum halides, or the Wurtz-Fittig reaction with sodium metal.

b. The halogenated compounds react with active metals to form organo-metallic derivatives.

c. The halogenated compounds react with active metal salts of alcohols, phenols, thiophenols, xanthates, phosphates, and thiophosphates, to produce varied derivatives.

Examples of the above are:

1. Alpha dichloro-di-p.-chlorophenyl azelate.
2. Zinc di-(alpha chloro-alpha thiophenyl) lauryl azelate.
3. Methyl dichloro-stearyl alpha-dichloro-tri-phenyltin azelate.
4. 2, 8-dichloro-2,8-ethylxanthyl calcium ricinoleyl azelate.
5. 2,8-dibromo-azeloyl lithium benzene p.-sulfonate.
6. Alpha-chloro-alpha-isopropylphenyl azeloyl-zinc distearate.
7. Alpha-chloro-alpha-dibutyl thiophosphato-lauryl naphthyl dithioazelate.

The metal salts of substituted azelaic acid, the halogen-bearing azelates show desirable oiliness or load-carrying properties, the metal salts of substituted acids possess detergent properties, and the sulfur, phosphorous, and nitrogen derivatives have antisludging, anticorrosion, and antioxidant properties.

Over and above these generally recognizable properties, we are able to add distinct and particular values by introducing:

a. Controlled oil solubility through the reactivity of the terminal carboxyl groups and the active carbon chain, through which selected alkyl or aryl oil solubilizing groups may be attached to the azeloyl group as a substituent in the chain or as a carboxyl derivative, or to the salt forming metal.

b. Controlled extreme pressure or oiliness properties due to the presence of two active carbons positioned adjacent to the carboxyl groups, by which means alpha-chloro or dichloro azelates may be formed which have been shown to have highly polar adsorptive properties to metals forming multimolecular oriented films of the addend on lubricated metal surfaces, such that a continuous effective lubricant film is maintained under conditions of boundary lubrication.

c. Controlled antisludging, anticorrosion, and anti-oxidation activity through the ability to introduce functional elements such as sulfur in optimum ratio in the molecule as, for example, one or more mercapto, sulfide, disulfide, polysulfide, thiocyanate, sulfoxide, sulfone groups, or as sulfur substituted organic radicals such as thiophosphate, xanthate, thiocarbonate or aryl-sulfonate.

The particularly advantageous feature of the combined oiliness and otherwise functional addend appears to lie in the ability of the alpha-halogenated oil-soluble addend to be adsorbed and oriented on the lubricated metal surface by which action the additional functional addend is, perforce, retained in the adsorbed film and, due to the normal carbon valence angles, held adjacent to the metal where the conditions for catalytic and thermal breakdown of the lubricant are at an optimum and precisely where the detergent, antioxidant, anticorrosive, or antisludging agent is needed to solubilize, peptize, or disperse such non-lubricant products of oil or fuel dissociation as may be formed, or inhibit the formation of oxidation and corrosion catalysts. Through the regulated synthesis of the preferred additive, the optimum ratio of detergency—oiliness—antioxidation—antifoaming and other selected properties may be instituted, or any preferred particular function or functions may be emphasized to the exclusion of others.

The procedure to be followed in the synthesis of the typical products contemplated by this invention will be made clear to one skilled in the

art by the following examples which are presented for the purposes of illustration:

*Example I*

Two parts of azelaic acid dissolved in four parts of a nonhalogenating solvent such as acetone is halogenated with chlorine gas in the liquid phase until the chlorine content attains thirty per cent of the reaction product (approximately 1.5 parts of chlorine being used). The chlorinated azelaic acid, having approximately the composition of the alpha-dichloride, is freed of the hydrogen chloride produced during halogenation and approximately 80 per cent of the neutral solvent by distillation at either atmospheric or reduced pressure. To this is added 1.0 part of potassium ethyl xanthate prepared by the action of alcoholic potassium hydroxide with carbon disulfide in the ratio of 1 part of potassium hydroxide to 4 parts of ethyl alcohol and 1.4 parts of carbon disulfide. The solution is warmed and refluxed four to five hours, after which the mixture is filtered to remove precipitated salts, and distilled to remove the solvent. The product is heated to 100° C. for one hour with 1 part of phosphorous trichloride and 1.8 parts of p-aminophenol, then poured into water, extracted with ether, recovered, washed, and dried. The product is then heated with 1 part of zinc oxide to 125° C. for one hour with stirring. The insoluble solids are removed by filtration, leaving an oil soluble zinc salt of alpha-chloro-alpha ethylxanthyl p-aminophenyl azelate, which may be dispersed or dissolved in the hydrocarbon lubricant to produce the preferred lubricant composition of our invention.

*Example II*

One part of ethyl xanthate and one part of n-butyl acid chloroazelate, prepared as described in Example I, are dissolved in two parts of acetone (or a similar alkyl ketone such as methyl-ethyl ketone) and refluxed for five hours. The solids are filtered off, washed with acetone, and the product recovered from the solvent. The mixed calcium salt of the substituted azelaic acid and stearic acid is prepared by the heating of two parts of the substituted azelaic acid with one part of stearic at 120-150° C. with alcoholic caustic for one hour. The clear solution is treated with a concentrated solution of calcium chloride which precipitates the mixed salt. The dehydrated metal salt is dissolved and/or dispersed in a SAE 50 mineral oil with heating, to serve as a concentrate for the preparation of the lubricant composition of our invention.

*Example III*

Five parts of sodium alpha-dichloro-azelate in ether solution, prepared as described in Example I, are treated with 5.5 parts of p-dichlorobenzene and two parts of finely divided sodium. The reaction proceeds vigorously at room temperature with the precipitation of solid NaCl. After the spontaneous reaction has subsided, the mass is refluxed four to six hours, acidified with dilute sulfuric acid, filtered, the residue washed with ether, the ether solutions united, and heated under reflux with four parts of sodium laurolate to produce the acid lauryl ester. The resulting products are then treated with 3.5 parts of triphenyltin hydroxide for three hours under gentle warming. The precipitated salts are filtered off, the product is recovered from ether, dried and suspended in a mineral oil to produce an additive concentrate for the preparation of the blended lubricant composition.

*Example IV*

Two parts of alpha dichloroazelaic acid, prepared as described in Example I, are boiled with one part of acetyl chloride to produce azeloyl anhydride. To this is added two parts of diphenyl methyl methoxy silane (prepared by the action of Grignard reagents on silicon tetrachloride and the subsequent treatment with sodium methylate) in ether solution. On gentle heating, the silico-ester is split forming the diphenyl methyl silico-methyl dichloro azelate, which is freed of ether by distillation. The product is dissolved in benzol or naphtha for the preparation of the preferred blended lubricant.

*Example V*

Two parts of alpha-dichloro-azelaic anhydride, prepared as described above, are treated with two parts of diphenyl methyl ammonium hydroxide in alcoholic solution. The mass is heated under reflux for two hours, then two parts of a ten per cent solution of lithium hydroxide are added with further heating and stirring. The reaction products are freed of alcohol, dried, and dissolved in a light lubricating oil with heating to 100° C. The lubricating oil concentrate of the additive is then used in preparing the blended lubricant composition.

*Example VI*

Five parts of alpha dichloro azelaic acid, prepared as illustrated in Example I, are treated with six parts of isopropyl-benzene and two parts of anhydrous aluminum chloride. The reaction is completed on heating to 120-150° C. for two hours. The product is mixed with 5.5 parts of oleic acid and three parts of milled, hydrated, barium oxide; the reaction mass is heated with stirring to 120-150° C. for three hours, after which the insolubles are removed by filtration and the oily brown liquid is treated with two parts of phosphorous pentasulfide with stirring for two hours at 150° C. The orange-brown oily product is filtered, clarified by contacting with filtrol clay, and prepared in an oil solution for the preparation of the preferred blended lubricant of our invention.

By way of example and not by way of limitation, the following examples of preferred lubricant additives are given. Additives inhibiting corrosion, oxidation and sludge formation in lubricants:

1. Sodium anilino-8-chloro 8-diethyl-thiophosphato-azelate.
2. Zinc di-(8,8'-dibutylthiophosphato) thiophenyl azelate.
3. Dithiofurfuryl 8-dithiobutyl thiophenyl azelate.
4. Thiophenyl 8-diethylthiophosphato-3,5-di-  
amylphenyl azelate.
5. Di-alpha-ethylxanthyl azeloyl triphenyl-  
silicon imide.
6. Lauryl diethylxanthyl thio-oleyl azelate.
7. Di-alpha-ethylxanthyl azeloyl disulfide.
8. Di-alpha-thiophenyl di-thio-octadecyl azelate.

Additives inhibiting foaming in lubricants:

1. Diphenyl lauryl-azeloyl-silic平 or its condensation product.
2. Diisobutyl di-phenylazeloyl silane or its condensation product.
3. Hexyl alpha-dibutylphosphato-methyl azeloyl silicon diol or its silicone condensation products.

4. Butyl di-phenyl tetramethylammonium alpha dichloroazetyl silicane or its condensation products.

Additives imparting detergent properties to a lubricant:

1. Zinc di (alpha-chloro alpha ethylxanthyl) p-amylophenyl azelate.

2. Stearyl-calcium di-ethylxanthyl butyl azelate.

3. Triphenyl-tin di-p-chlorophenyl lauryl azelate.

4. Lithium diphenyl methyl ammonium alpha dichloro azelate.

5. Barium diisopropylphenyl azelate thiophosphate-oleate.

6. Lithium alpha-chloro alpha-ethylxanthyl butyl azelate.

7. Bismuth 8,8' butylxanthyl ethyl azelate alpha dichloro-stearate.

8. Zinc di (8,8'-dibutyl thiophosphato) thiophenyl azelate.

9. Calcium di (dibenzyl) azelate.

10. Methyl lauryl alpha diphenyl p-calcium sulfonate.

11. Calcium di (alpha di-cresyl) triamyl-silicon amido-azelate.

12. Barium di (di-alpha ethylxanthyl) stearyl azelate.

13. Lithium alpha dithiophenyl thiocresyl azelate.

14. Cadmium (di-alpha phenyl-p-cadmium sulfonate) azelate.

15. Lithium alpha-diphenyl p-chlorophenyl dithio-azelate.

Metals other than those illustrated above may be used in salt formation such, for example, as:

|           |           |
|-----------|-----------|
| Sodium    | Cobalt    |
| Lithium   | Zinc      |
| Potassium | Nickel    |
| Magnesium | Manganese |
| Calcium   | Aluminum  |
| Strontium | Chromium  |
| Lead      | Tin       |
| Copper    | Cadmium   |
| Bismuth   | Silver    |
| Mercury   | Tellurium |
| Barium    |           |

Additives imparting extreme pressure characteristics to the lubricant:

1. Di-p-chlorophenyl alpha dichloro-azelate.

2. Lauryl alpha dichloro methyl azelate.

3. Diphenyl-ammonium alpha-dichloro alpha-naphthyl azelate.

4. Alpha-dichloro-stearyl bismuth alpha-di-chloro thiophenyl azelate.

5. Cyclohexyl 8-chloro 8-ethylxanthyl phenyl azelate.

6. Alpha dichloro methyl azetyl phenyl hydrazide.

7. Calcium di-(alpha-chloro alpha-thiophenyl) lauryl azelate.

8. Zinc di-(alpha-chloro alpha-ethylxanthyl) p-amylophenyl azelate.

Additives imparting oiliness characteristics to the lubricant:

1. Methyl 2,2 dichloro 8,8-thiophenyl lauryl azelate.

2. Methyl 2,2-dichloro 8,8-ethylxanthyl thiophenyl azelate.

3. Methyl alpha-dithiophenyl thiocresyl azelate.

4. Diamylphenyl 2,8-dichloro 2,8-di-diethyl-thiophosphate-lauryl azelate.

5. Butyl 2-dichloro 8-dithiophenyl methyl azelate.

If the compounded lubricant is to be used under high temperature conditions the addition agent should be nonvolatile and stable at elevated temperatures. For example, if the lubricant is to be used in the crankcase of an internal combustion engine the additive must have a boiling point above 150° F. and must not dissociate from the lubricant at temperatures as high as 250° F.

It is sometimes desirable to provide the addition agents in the form of a concentrate in a suitable oil. Such concentrates may be employed for further blending with a blended lubricating oil in the proportion desired for the particular conditions of use.

The additive may be blended with mineral lubricating oils or with other oils of lubricating viscosity such as vegetable oils, animal oils, synthetic oils or light oil distillates. Furthermore, it is not essential that the additive be the only ingredient in the lubricant; it being understood, of course, that no additional ingredient should be present which is incompatible with the addition agent. Other additives such as those commonly used to improve viscosity index or cold test may be used also.

When used with a blended hydrocarbon oil, only such amounts of the additive should be incorporated as are soluble in the specified amount of oil. By the term "soluble," it is intended to indicate the ability to form not only true solutions but also any form of substantially permanently homogeneous composition when incorporated in a blended mineral oil base. Since quite small percentages often give remarkably improved results, it is seldom of extreme importance that the addition agent be oil soluble in all proportions.

It will be understood that certain features and sub-combinations are of utility and may be employed without reference to other features and subcombinations. This is contemplated by and is within the scope of our claims. Various changes in details may be made without departing from the spirit of our invention.

Having thus described our invention, we claim:

1. A lubricant comprising a major proportion of an oil of lubricating viscosity having a minor proportion, sufficient to improve the lubricating characteristics of the oil, of an aliphatic diacid of from 6 to 12 carbon atoms, said acid having terminal carboxyl groups which are substituted with a silicon containing radical.

2. A lubricant comprising a major proportion of an oil of lubricating viscosity having a minor proportion, sufficient to improve the lubricating characteristics of the oil, of halogen substituted aliphatic diacid of from 6 to 12 carbon atoms having terminal carboxyl groups which are substituted with a silicon containing radical.

3. A lubricant comprising a major proportion of an oil of lubricating viscosity and a minor proportion, sufficient to improve the lubricating characteristics of the oil, of azelaic acid, the terminal carboxyl groups of which are substituted with at least one chemical group which contains silicon.

4. A lubricant comprising a major proportion of an oil of lubricating viscosity and a minor proportion, sufficient to improve the lubricating characteristics of the oil, of a salt of azelaic acid, the terminal carboxyl groups of which are substituted with at least one silicon-containing chemical group.

5. A lubricant comprising a major proportion

of an oil of lubricating viscosity and a minor proportion, sufficient to improve the lubricating characteristics of the oil, of a metal salt of azelaic acid, the terminal carboxyl groups of which are substituted with at least one silicon-containing chemical group.

6. A lubricant comprising a major proportion of an oil of lubricating viscosity and a minor proportion, sufficient to improve the lubricating characteristics of the oil, of an amine salt of azelaic acid, the terminal carboxyl groups of which are substituted with at least one silicon-containing chemical group.

7. A lubricant comprising a major proportion of an oil of lubricating viscosity and a minor proportion, sufficient to improve the lubricating characteristics of the oil, of an ammonium salt of azelaic acid, the terminal carboxyl groups of which are substituted with at least one silicon-containing chemical group.

8. A lubricant comprising a major proportion of an oil of lubricating viscosity and a minor proportion, sufficient to improve the lubricating characteristics of the oil, of an ester of azelaic acid, the terminal carboxyl groups of which are substituted with at least one silicon-containing chemical group.

10

9. A lubricant comprising a major proportion of an oil of lubricating viscosity and a minor proportion, sufficient to improve the lubricating characteristics of the oil, of a metal ester of

5 azelaic acid, the terminal carboxyl groups of

which are substituted with at least one silicon-

containing chemical group.

15

BERT H. LINCOLN.  
JOSEPH M. HERSH.

## REFERENCES CITED

The following references are of record in the file of this patent:

15

## UNITED STATES PATENTS

| Number    | Name              | Date           |
|-----------|-------------------|----------------|
| 2,349,817 | Farrington et al. | May 30, 1934   |
| 2,334,158 | Fuchs et al.      | Nov. 9, 1943   |
| 2,330,239 | Prutton           | Sept. 28, 1943 |
| 2,280,474 | Byrkit et al.     | Apr. 21, 1942  |
| 2,262,773 | Lincoln et al.    | Nov. 18, 1941  |
| 2,329,474 | Lazar et al.      | Sept. 14, 1943 |

25

## FOREIGN PATENTS

| Number  | Country | Date         |
|---------|---------|--------------|
| 500,222 | British | Feb. 6, 1939 |